

1

3,175,902

## AUSTENITIC ALLOY

Joseph A. Ferree, Jr., Natrona Heights, Pa., assignor to Allegheny Ludlum Steel Corporation, Brackenridge, Pa., a corporation of Pennsylvania  
 No Drawing. Filed Nov. 6, 1962, Ser. No. 235,867  
 6 Claims. (Cl. 75—128)

This invention relates to fully austenitic stainless steel and in particular to fully austenitic stainless steels which are characterized by having a constant density within given limits and which are particularly suited for use as mass standards.

At the present time, there is no standard weight material. Brass which has often been employed has numerous disadvantages in that it is not resistant to corrosion and, consequently, may show significant variations in mass with time because of oxidation and/or corrosion. In addition, brass has a low resistance to abrasion and may lose some weight in use. In order to alleviate these conditions, resort has been sometimes had to gold plating of the brass mass standards in order to overcome the corrosion and oxidation problems. However, gold plate also has a low abrasion resistance and in some instances, the gold plate may exhibit surface imperfections which may cause accelerated corrosive attack by galvanic action with the base metal.

Variations in density due to differences in composition, unsoundness, dissolved gases and non-metallic inclusions are other sources of inaccuracies. Moreover, differences in density readily complicate calibration of mass standards because the buoyancy effects of the atmosphere will be different for standards with the same mass but different volumes. In order to attain some uniformity for mass standards the National Bureau of Standards has proposed a number of requirements which must be met for a material to be used as an optimum mass standard. These requirements include:

- (1) Sufficient abrasion resistance to prevent loss in mass during regular, careful usage.
- (2) The material must have the ability to be polished to a mirror finish.
- (3) The material must be non-magnetic.
- (4) The material must be resistant to atmospheric corrosion and oxidation to avoid the necessity for plating; and
- (5) The material must have a constant uniform density of  $8.0 \pm 0.1$  g./ml. at  $25^\circ C$ .

The fully austenitic steel of the present invention meets the requirements set forth by the National Bureau of Standards.

An object of this invention is to provide a fully austenitic stainless steel suitable for use as a mass standard.

Another object of this invention is to provide a fully austenitic steel having a preferred balanced composition within given limits to provide a density within the range between  $8.0 \pm 0.1$  g./ml. at  $25^\circ C$ .

A more specific object of this invention is to provide an iron-chromium-nickel-molybdenum fully austenitic stainless steel having good abrasion resistance and a balanced composition to provide a constant uniform density of  $8.0 \pm 0.1$  g./ml. at  $25^\circ C$ .

Other objects of this invention will become apparent to those skilled in the art when taken in conjunction with the following description.

The steel of the present invention in its broader aspects contemplates a composition which includes up to 0.10% carbon maximum, from 1.0% to 2.0% manganese, up to 0.03% maximum phosphorus, up to 0.03% maximum sulfur, from about 0.25% to about 1.0% silicon, from about 17.5% to about 22.5% chromium, from about

2

23.0% to about 27.5% nickel, from about 1.0% to about 3.25% molybdenum, optional to about 1.5% maximum tungsten, optional to about 0.5% maximum copper and the balance substantially iron with incidental impurities.

5 Each of the elements present within the composition set forth within the broad ranges enumerated hereinbefore performs a specific function. While carbon is present up to a maximum of 0.10%, it is preferred to maintain the carbon content as low as possible within reasonably commercial melting practices. This results from the fact that it is desirable to afford the steel with a maximum amount of corrosion resistance and the utilization of low amounts of carbon are effective for providing the maximum amount of chromium for optimum corrosion resistance.

Manganese is present for conferring hot workability to the steel of the present invention and in this respect, it should be noted that manganese will also combine with certain gases to thereby reduce the amount thereof thus 10 removing one of the inaccuracies resulting in variations in density. It is preferred to have at least 1.0% manganese present and the addition of more than about 2.0% does not appear to be beneficial. Optimum results have been obtained where the manganese content is maintained 15 within the range between about 1.25% and about 1.75%.

Silicon is preferably present within the range between 0.25% and about 1.0% and acts in conjunction with the manganese in aiding the fabrication of the steel and in removing the amount of occluded gases. Preferably the 20 silicon content does not exceed about 1.0%. Optimum results have been obtained where the silicon content is maintained 25 within the range of 0.4% and 0.6%.

Chromium is present within the steel of the present invention in a minimum amount of 17.5% in order to obtain the required degree of corrosion resistance. White 30 chromium can be present up to about 22.5%, it is preferred not to exceed this upper limit in order to insure freedom from the presence of delta ferrite within the microstructure thus insuring that the steel will have a minimum magnetic permeability. Where the chromium content is maintained within the optimum range of about 19.0% to about 21.0%, the steel is afforded a combination of a maximum degree of corrosion resistance consistent with constant magnetic permeability and a control 35 of the density to within  $\pm 0.05$  g./ml. from the ideal density of about 8.0 g./ml. where the balance of the alloying components are proportioned as will be described 40 hereinafter.

The steel of the present invention contains between 45 23.0% and 27.5% nickel, which functions to insure a fully austenitic structure which is characterized by having an austenite stability which will prevent any possible transformation of the non-magnetic austenite to magnetic martensite during such operations as machining, polishing and subsequent usage. The optimum austenite stability is obtained where the nickel content is maintained 50 within the range between 24.0% and about 26.0%. Moreover, nickel together with chromium aids the corrosion resistance.

60 The steel of the present invention utilizes molybdenum in the minimum amount of 1.0% whereas the maximum should not exceed about 3.25%. The element molybdenum confers a high degree of corrosion resistance especially where the atmosphere may contain one of the halogen elements. Molybdenum also contributes to the abrasion resistance of the steel and is particularly useful for balancing the composition with respect to obtaining the required density since the element molybdenum has a relatively high density. In this respect, it should be noted 65 that it is possible to substitute up to approximately 1.5% maximum tungsten for the molybdenum. While tung-

sten is also effective for providing the steel with an increased measure of resistance to abrasion, none the less, it does not provide the additional corrosion resistance which is obtainable through the use of molybdenum. Accordingly, it is preferred that the steel of the present invention utilize molybdenum in preference to tungsten. Optimum results appear to be obtained where the molybdenum content is maintained within the range between about 1.25% and about 2.75%.

Copper may also be present within the steel of the present invention; however, it is preferred to limit the copper content to about 0.5% maximum. Normal melting operations are usually effective for obtaining low copper contents and preferably the copper should not be in excess of about 0.2%.

The balance of the steel is substantially iron with the normal amounts of phosphorus and sulfur which it is preferred to maintain at the minimum. In this same respect, it is also desired to maintain the other incidental impurities such as dissolved oxygen and nitrogen at a minimum in order to obtain the highest quality of material.

As stated hereinbefore, freedom from dissolved gases, unsoundness and non-metallic inclusions is required in order to minimize the amount of inaccuracies and variations in density. Consequently, it is preferred to vacuum melt the steel of the present invention. This may be conveniently accomplished through the utilization of vacuum induction melting and further refinements of the steel are possible by utilizing the vacuum melted material as a consumable electrode for the production of consumable electrode vacuum remelt material. By thus utilizing the foregoing melting techniques which are common in the art, it is possible to minimize the inaccuracies due to non-metallic inclusions, dissolved gases and unsoundness of the finally produced product. It should be noted, however, that the melting practice per se is not a limitation on the steel of the present invention and where desired other melting practices may be employed in order to obtain the steel of the present invention.

Reference is respectfully directed to Table I which illustrates the chemical composition of the steel of the present invention, it being noted that Table I contains the limits for the general range as well as the preferred range of composition.

TABLE I  
Chemical composition

[Percent by weight]

| Element        | General Range | Preferred Range |
|----------------|---------------|-----------------|
| C              | 0.10 max.     | 0.03 max.       |
| Mn             | 1.0-2.0       | 1.25-1.75       |
| P              | .03 max.      | .03 max.        |
| S              | .03 max.      | .03 max.        |
| Si             | .025-1.0      | 0.4-0.6         |
| Cr             | 17.5-22.5     | 19.0-21.0       |
| Ni             | 23.0-27.5     | 24.0-26.0       |
| Mo             | 1.0-3.25      | 1.25-2.75       |
| W <sup>1</sup> | 1.5 max.      | 1.25 max.       |
| Cu             | 0.5 max.      | 0.2 max.        |
| Fe             | Bal.          | Bal.            |

<sup>1</sup> Optional to stated limit with a corresponding percent decrease in molybdenum.

As was stated hereinbefore, the steel of the present invention finds particular usage as a constant density alloy in the fabrication of mass standards. These standards require that the steel have a constant uniform density of  $8.0 \pm 0.1$  g./ml. at  $25^\circ C$ . However, in order to be commercially feasible, it was necessary to devise a procedure for predicting the final density of a melt prior to tapping while adjustments in the analysis can be made. This resulted from the fact that certain combinations of the alloying elements within the range set forth hereinbefore in Table I would not produce densities within the required limits.

Experimental procedures resulted in deriving an em-

pirical formula specifically for the range of analysis set forth in Table I which will assure a density within the limits of  $8.0 \pm 0.1$  g./ml. at  $25^\circ C$ . This empirical formula enables the adjustment of the chemistry of the steel prior to tapping and will insure the final production to have the required density. The empirical formula is as follows:

formula is as follows:

$$\text{Density} = 0.001415 [(\% \text{Fe}) (55.85) + (\% \text{Mn}) (54.93) + (\% \text{Si}) (28.06) + (\% \text{Cr}) (52.01) + (\% \text{Ni}) (58.69) + (\% \text{Mo}) (95.95) + (\% \text{W}) (183.92) + (\% \text{Cu}) (63.54)]$$

It is to be noted that the empirical formula set forth does not contain any provisions for such elements as carbon, nitrogen, phosphorus and sulfur. Since these elements are fairly low and are also fairly constant their effect on the density is negligible.

Moreover, the effect on density of the elements manganese, silicon and chromium which have atomic weights less than that of iron are inversely proportional to the weight percentage. Thus when the percentages of these elements are high, the density decreases yet the total effect is still additive and must be considered in conjunction with the balance of the alloying elements there present. Consequently, when slight variations in the adjustment of the final chemistry are necessary it must be kept in mind that the addition of manganese, silicon and chromium will reduce the calculated density whereas the addition of such elements nickel, molybdenum, tungsten and copper increases the density. Thus, from the foregoing empirical formula which relates only to the steel of this invention within the limits set forth hereinbefore, the final density can be predicted within the limits set forth through the balance of the chemical composition of each of the alloying components.

In order to more clearly demonstrate the steel of the present invention, reference is directed to Table II which contains the identity of three heats which were made and tested following the teachings of the present invention. These steels have the composition set forth in Table II and the utilization of the empirical formula set forth hereinbefore forms the basis for the recorded data for the theoretical density. The actual density measurements in g./ml. at  $25^\circ C$ . are also set forth showing the close agreement between theoretical and actual density.

TABLE II

| Element             | Heat X | Heat C | Heat N |
|---------------------|--------|--------|--------|
| C                   | .092   | .093   | .0097  |
| Mn                  | 1.44   | 1.49   | 1.46   |
| Si                  | 0.54   | 0.53   | 0.40   |
| P                   | 0.024  | 0.021  | 0.010  |
| S                   | 0.018  | 0.021  | 0.013  |
| Cr                  | 20.02  | 19.84  | 20.29  |
| Ni                  | 24.88  | 25.05  | 25.54  |
| Mo                  | 2.07   | 2.05   | 2.38   |
| W                   | 0.13   |        |        |
| Cu                  | 0.20   | 0.16   | 0.20   |
| N                   | 0.024  | 0.030  |        |
| Fe                  | 50.68  | 50.58  | 49.68  |
| Theoretical Density | 7.98   | 8.0    | 7.99   |
| Actual Density      | 7.98   | 8.0    | 8.01   |

Steel from the foregoing heats was readily fabricated into bars by hot rolling, there being no difficulty encountered. Thereafter pieces from the bars were machined, diamond burnished by the method described by E. H. Hull "Machinery," January 1962, pages 92 through 97, which is in accordance with the requirements set forth by the National Bureau of Standards, and polished with 600 grit silicon carbide paper for testing. Measurement of the actual density as recorded in Table II compared exceedingly well with the theoretical density calculations made by utilizing the empirical formula set forth hereinbefore. Thus, with the close control and agreement of the actual density with the theoretical density, the initial

requirement of the material having the controlled density is adequately met. Accordingly, the empirical formula set forth hereinbefore becomes a practical means for controlling the chemistry of the composition in order to obtain a steel having a predetermined density.

Additional samples from Heat N after diamond burnishing were measured for surface roughness. As diamond burnished, Heat N exhibited a profilometer reading of 5.6 R.M.S. microinches. Thereafter, the bar material was polished with 600 grit silicon carbide paper, and again using a profilometer, the surface roughness measurements exhibited by the bar decreased to 0.8 R.M.S. microinch. The National Bureau of Standards has indicated that a surface roughness of 1.2 R.M.S. microinches is quite satisfactory. As indicated, the steel of the present invention easily meets this capability. Further tests were run on Heat N, which included surface hardness. These test results, converted into a Brinell Hardness Number from the Rockwell 15-T, demonstrated a hardness equivalent to 185 BHN. This hardness was for material in the annealed condition after diamond burnishing and polishing. Contrasted thereto, cold worked material exhibited a hardness of over 200 BHN, depending upon the amount of cold work. By comparison, annealed gold exhibits a hardness of about 25 BHN, and brass about 60 BHN, thus indicating the outstanding hardness and abrasion resistance exhibited by the steel of the present invention in comparison with both gold and brass which have been heretofore used as constant mass standards.

Heat N was also subjected to a measurement of its magnetic permeability in the annealed condition, as well as in the cold worked condition in order to determine the stability of the austenite. These measurements indicated that Heat N exhibited a magnetic permeability of less than 1.005 at 200H. After heavy cold reductions, no magnetic phases were detected. Since Magna gauge tests on the surface of the polished bar indicated a permeability of less than 1.005, which is the lowest limit as respects the sensitivity of the Magna gauge in measuring the magnetic permeability, it is clear that the present alloy possesses a high degree of austenite stability.

The most stringent characteristic of a constant mass standard relates to its corrosion resistance. Material from Heat N was also subjected to the standard corrosion resistance test which simulates conditions to be normally found in the careful usage of such a material as a constant mass standard. Samples from Heat N were cleaned with 20% nitric acid at room temperature to remove any contaminants which may have been present after burnishing and polishing. Samples were exposed to 100% relative humidity at a temperature within the range of from 100 to 125° F. After four days' exposure there was no corrosive attack or discoloration noted. These same samples were also exposed to 100% relative humidity at room temperature for three days without any detectable changes having occurred. Thereafter these same samples were tested in 5% neutral salt spray for a period of eight days. After eight days the material was again examined, and there was no visible corrosive attack, discoloration or any other adverse effect noted from this test.

No special skills are required in producing this alloy, and regular commercial mill equipment was utilized in the production thereof.

I claim:

1. A constant density alloy consisting essentially of up to 0.10% carbon, from 1.0% to 2.0% manganese, from 0.25% to 1.0% silicon, from 17.5% to 22.5% chromium, from 23.0% to 27.5% nickel, from 1.0% to 3.25% molybdenum and the balance essentially iron with incidental impurities and which is characterized by exhibiting

a constant density within the range between 7.9 and 8.1 g./ml. at 25° C.

2. A constant density alloy consisting essentially of up to 0.03% carbon, from 1.25% to 1.75% manganese, from 0.40% to 0.60% silicon, from 19.0% to 21.0% chromium, from 24.0% to 26.0% nickel, from 1.25% to 2.75% molybdenum and the balance essentially iron with incidental impurities and which is characterized by exhibiting a constant density within the range between 7.95 and 8.05 g./ml. at 25° C.

3. A fully austenitic stainless steel particularly suited for use as a constant mass standard consisting essentially of up to 0.10% carbon, from 1.0% to 2.0% manganese, from 0.25% to 1.0% silicon, from 17.5% to 22.5% chromium, from 23.0% to 27.5% nickel, from 1.0% to 3.25% molybdenum, optional to 1.5% tungsten, optional to 0.5% copper and the balance essentially iron with incidental impurities, and which is characterized by exhibiting a density  $\delta$  within the range between 7.9 and 8.1 g./ml. at 25° C. resulting from balancing the constituents of the alloy within the ranges stated according to the following formula:

$$\delta = 0.001415 [(\% \text{Fe}) (55.85) + (\% \text{Mn}) (54.93) + (\% \text{Si}) (28.06) + (\% \text{Cr}) (52.01) + (\% \text{Ni}) (58.69) + (\% \text{Mo}) (95.95) + (\% \text{W}) (183.92) + (\% \text{Cu}) (63.54)]$$

4. A fully austenitic stainless steel particularly suited for use as a constant mass standard consisting essentially of up to 0.03% carbon, from 1.25% to 1.75% manganese, from 0.40% to 0.60% silicon, from 19.0% to 21.0% chromium, from 24.0% to 26.0% nickel, from 1.25% to 2.95% molybdenum, optional to 1.25% tungsten, optional to 0.2% copper and the balance essentially iron with incidental impurities, and which is characterized by exhibiting a density  $\delta$  within the range between 7.95 and 8.05 g./ml. at 25° C. resulting from balancing the constituents of the alloy within the ranges stated according to the following formula:

$$\delta = 0.001415 [(\% \text{Fe}) (55.85) + (\% \text{Mn}) (54.93) + (\% \text{Si}) (28.06) + (\% \text{Cr}) (52.01) + (\% \text{Ni}) (58.69) + (\% \text{Mo}) (95.95) + (\% \text{W}) (183.92) + (\% \text{Cu}) (63.54)]$$

5. A constant mass standard formed from a fully austenitic stainless steel having a composition consisting essentially of up to 0.10% carbon, from 1.0% to 2.0% manganese, from 0.25% to 1.0% silicon, from 17.5% to 22.5% chromium, from 23.0% to 27.5% nickel, from 1.0% to 3.25% molybdenum, optional to 1.5% tungsten, up to 0.5% copper, and the balance essentially iron with incidental impurities, characterized in that each of the constituents of the metal is balanced to provide the mass standard with a density within the range between 7.9 and 8.1 g./ml. at 25° C.

6. A constant mass standard formed from a fully austenitic stainless steel having a composition consisting essentially of up to 0.03% carbon, from 1.25% to 1.75% manganese, from 0.4% to 0.6% silicon, from 19.0% to 21% chromium, from 24% to 26% nickel, from 1.25% to 2.75% molybdenum, optional to 1.25% tungsten, up to 0.2% copper, and the balance essentially iron with incidental impurities, characterized in that each of the constituents of the metal is balanced to provide the mass standard with a density within the range between 7.95 and 8.05 g./ml. at 25° C.

#### References Cited by the Examiner

#### UNITED STATES PATENTS

2,606,113 8/52 Payson et al. \_\_\_\_\_ 75—128.9

70 DAVID L. RECK, Primary Examiner.